

Nov. 10, 1936.

O. R. RICE

2,060,346

TUYERE

Original Filed Oct. 22, 1934 2 Sheets-Sheet 1



Fig. 7



Fig. 8



Fig. 9



Fig. 1



Fig. 6



Fig. 2



Fig. 3



Fig. 4

Fig. 5

BY

INVENTOR.  
OWEN R. RICE.

Wilkinson, Hulley, Bryant & Knight  
ATTORNEYS

Nov. 10, 1936.

O. R. RICE

2,060,346

TUYÈRE

Original Filed Oct. 22, 1934 2 Sheets-Sheet 2



Fig. 10



Fig. 11



Fig. 13



Fig. 12



Fig. 14

INVENTOR.  
OWEN R. RICE.

BY

William H. Hulley, Byrum & Wright  
ATTORNEYS

## UNITED STATES PATENT OFFICE

2,060,346

## TUYÈRE

Owen R. Rice, Chicago, Ill., assignor to Freyn  
Engineering Company, Chicago, Ill., a corpora-  
tion of Maine

Original application October 22, 1934, Serial No.  
749,371. Divided and this application May 2,  
1935, Serial No. 19,431

## 4 Claims. (Cl. 266—41)

The present invention relates to improvements in methods of casting.

More particularly the present invention relates to the method of casting rigid blocks within metal 5 having a different coefficient of expansion than said blocks. The present invention is particularly useful in the manufacture of tuyères having refractory noses, and will be described in connection with tuyères.

10 This application is a division of application Serial No. 749,371, filed October 22, 1934, by the present applicant.

An object of the present invention is to simplify the manufacture of castings having preformed 15 rigid blocks located therein.

A further object is to provide an improved method of making a casting having a circular assembly of preformed blocks located therein.

20 A further object is to provide an improved method of making a tuyère embodying preformed refractory blocks in the nose thereof.

Further objects will appear as the description proceeds.

## Referring to the drawings—

25 Figure 1 is a view in end elevation showing the nose portion of a tuyère embodying the principles of the present invention, illustrating particularly the disposition of refractory blocks within the nose portion of the tuyère;

30 Figure 2 is a fragmentary sectional view taken along the plane indicated by the arrows 2—2 of Figure 1;

35 Figure 3 is a view similar to Figure 2 but showing an alternative construction for holding the refractory blocks in place;

Figures 4 and 5 are views in end elevation and side elevation, respectively, of the block appearing in Figure 2;

40 Figure 6 is a view in end elevation of the block appearing in Figure 3;

Figure 7 is a fragmentary view similar to Figure 1 but showing the arrangement of preformed refractory blocks for a different diameter of tuyère;

45 Figure 8 shows the arrangement of blocks for another diameter of tuyère;

Figure 9 shows the arrangement of blocks for another diameter of tuyère;

50 Figure 10 shows the arrangement of blocks for still another diameter of tuyère;

Figure 11 illustrates the method of spacing the refractory blocks preparatory to the operation of casting the tuyère;

Figure 12 is a fragmentary elevational view of the structure shown in Figure 11;

Figure 13 is a view illustrating how a portion of a shim may remain after the casting operation; and

Figure 14 is a fragmentary elevational view of the structure shown in Figure 13.

The present invention has been illustrated in connection with a tuyère of the type generally known as water-cooled. By reference to Figure 2 it will be noted that the tuyère comprises the inner cone wall 10, the outer cone wall 11, and the front wall 12. Said walls, together with a back wall (not illustrated), form a jacket for cooling medium, usually water, through which the cooling medium may flow in a continuous stream to carry away heat from the metal of the tuyère.

Extending forwardly from the front wall 12 are the inner annular rib or fin 13 and the outer annular rib or fin 14, which ribs or fins 13 and 14 are disposed coaxially of the tuyère. In the outwardly opening recess between the front wall 12 and the annular ribs 13 and 14 are a plurality of preformed segmental blocks 15—15, which blocks, in order that they may fit approximately around the circumference of a circle, have side faces tapering toward one another.

In the manufacture of a tuyère embodying the principles of the present invention, the copper of the tuyère is cast around the preformed refractory blocks 15—15. According to the construction illustrated in Figure 2, a dove-tailed 30 tenon 16 is provided, which tenon extends circumferentially of the tuyère in the space provided by the wall 12 and the annular ribs or fins 13 and 14.

In the construction illustrated in Figure 3, 35 the faces of the refractory blocks 15—15 which face the axis of the tuyère are provided with a pair of holes 17—17. These holes are disposed at an angle one to the other so that when they are filled up with copper in the casting operation to form lugs, indicated by the numerals 17a—17a, the blocks are held firmly in a manner comparable to the "toe-nailing" of a board. In either of the constructions illustrated in Figures 2 and 3, the copper side walls or ribs 13 and 14 45 may burn away in service, but the blocks are securely held either by the tenon 16 or the lugs 17a—17a within the holes 17—17, which tenons or lugs are themselves an intimate part of the cool water wall of the tuyère body. In the construction illustrated in Figure 3, a vent 18 is provided communicating with each pair of holes 17—17, whereby to facilitate the casting operation.

In casting copper about a preformed rigid core, difficulty will be encountered in the case of certain preferred refractory cores due to the tendency of the copper to split upon cooling. This is because the coefficient of expansion of copper is higher than that of the preformed core. Moreover, since tuyères are made in many sizes, it would be necessary to have on hand many sizes of cores. In order to simplify the matter of stocking cores, and for the further purpose of overcoming the difficulty of splitting of the copper upon cooling, the present invention contemplates the use of a plurality of segmental preformed blocks which can be disposed circularly to form a core of any preferred diameter, within limits. Figure 1 shows a core made up of nine full blocks 15 and one cut block, the cut block being indicated by the numeral 19. In the operation of casting the tuyère, shims 20-20 (Fig. 11) of volatile substance, such as wood or paper, may be located between the blocks to permit the copper to contract upon cooling. The fact that the adjacent sides of the blocks do not make flat contact in certain cases is of no consequence. These spaces will be filled with intrusions or fins of cast copper, indicated by the numerals 21-21 (Fig. 13), which will serve the better to hold the blocks in place. In case the shims are not completely volatilized, no harm will result. Fragments of such shims are indicated by the numerals 20a-20a in Figure 13.

Figures 7, 8, 9 and 10 indicate relative positions of blocks such as shown in Figure 1, but for tuyères of different diameters.

By reason of the fact that the refractory is cast within the tuyère in the form of a plurality of preformed blocks, it is a simple matter to provide for the casting of different sizes of tuyères as required, and, further, it is a simple matter to provide for the differences in the coefficient of

expansion of the copper and the blocks, whereby the blocks may move in the cooling operation to allow contraction of the copper while cooling, whereby to avoid splitting of the copper.

The present disclosure is of course subject to modification. It is intended to cover all such modifications that fall within the scope of the appended claims.

What is claimed is—

1. The method of making a casting having rigid blocks therein which consists of disposing said blocks in proximity to one another but spacing them apart with volatile solid material and casting the molten metal about said rigid blocks and said volatile solid material. 15

2. The method of making a casting having a circular assembly of rigid blocks therein which consists in setting up a plurality of such blocks in a circular formation, spacing said blocks apart by means of volatile solid material, and casting 20 the molten metal about said blocks and said volatile solid material.

3. The method of making a blast furnace tuyère having a refractory nose which comprises setting up in a circular formation a plurality of rigid blocks tapering toward the axis of said circular formation, spacing said blocks apart by means of solid material volatile in molten metal, and casting molten metal around said rigid blocks and said volatile solid material. 25

4. The method of forming a tuyère having a refractory nose which comprises setting up a plurality of refractory blocks in a circular formation while spacing said blocks apart by means of volatile solid material and casting the nose portion of said tuyère around said blocks by pouring molten metal around said blocks, keying said blocks to said nose portion in the casting operation. 35

OWEN R. RICE. 40